

Aug. 18, 1959

F. J. O. W. OHLSSON

2,899,739

SINTERED HARD METAL ALLOY

Filed June 11, 1957



INVENTOR

FALL Johan Olof William Ohlsson

By Pierce, Scheffler & Parker  
Attorneys

1

2,899,739

## SINTERED HARD METAL ALLOY

Fall Johan Olof William Ohlsson, Enskede, Sweden, assignor to Sandvikens Jernverks Aktiebolag, Sandviken, Sweden, a corporation of Sweden

Application June 11, 1957, Serial No. 664,943

6 Claims. (Cl. 29—182.7)

The present invention relates to a sintered hard metal alloy of the well known type consisting essentially of tungsten carbide and titanium carbide (with or without a content of tantalum and/or niobium carbide) and an auxiliary or bonding metal selected preferably from the iron group of the periodic table, for instance cobalt, nickel and/or iron, and which has a structure built up of the following phases:

$\gamma$ -Phase consisting of a solid solution of WC and TaC/NbC (if present) in TiC,  $\beta$ -phase consisting of auxiliary or bonding metal (hereinafter called "bonding metal"), usually Co and/or Ni, and  $\alpha$ -phase consisting of WC.

For machine tool cutters for the finishing of steel, hard metal alloys have been used consisting of 5-7% by weight Co and a high TiC content, for example 20-36% by weight. In some cases a small amount of TaC has been included in the alloy. As an example of known alloys for this purpose I mention below the approximate proportions of two main types:

|     | A, percent by weight | B, percent by weight |
|-----|----------------------|----------------------|
| TiC | 25                   | 36                   |
| TaC | 6                    | 2                    |
| Co  | balance              | balance              |
| WC  |                      |                      |

The alloys of the type A have relatively satisfactory strength qualities, while their wear resistance is considerably lower than that obtainable by the alloys of the type B, the latter, however, having the drawback of being very fragile.

The object of the present invention is to produce a sintered hard metal alloy which has the qualities both of satisfactory strength and of satisfactory wear resistance. Alloys according to the present invention have been found to be particularly suitable for machine tools for finishing materials like steel giving long chips, but are not limited to this particular application.

A sintered hard metal alloy according to the present invention is defined both by the percentages of its components present in the alloy, and by a relationship between the amounts of the  $\beta$ - and  $\gamma$ -phases in the alloy.

Taking first the components of the alloy, a sintered hard metal alloy according to the present invention contains 30-45% by weight TiC, 1-5% by weight TaC/NbC and 8-13% by weight of bonding metal such as Co, Ni and/or Fe, the remainder being substantially all WC, although, as known in this art, other alloy components, for example, one or more of the carbides of molybdenum, chromium, vanadium and zirconium may be present in small amounts without disadvantage to the essential properties of the alloy. Furthermore, of course, whether or not these alloy components are present, the alloy of the invention is likely to contain certain impurities; thus, for example, the components TaC/NbC used for hard metal

2

alloys always contain small (insignificant) amounts of oxygen and nitrogen, and WC sometimes may contain small (insignificant) amounts of molybdenum carbide.

A sintered hard metal alloy according to the present invention is also characterized in that the amount of the  $\beta$ -phase of the alloy and the amount of the  $\gamma$ -phase are related to one another by the relationship

$$100 - \beta \geq \gamma > 100 - 2\beta$$

10 wherein  $\beta$  and  $\gamma$  represent the amounts of the respective phases expressed in volume percent. Preferably

$$\gamma > 100 - 1.5\beta$$

Any tendency to deformation of the cutting edge which 15 may occur with high bonding metal contents when using high cutting speed which give rise to high temperatures, can effectively be counteracted by means of an addition of TaC/NbC.

It should be here mentioned that where in this specification and the accompanying claims I refer to the alloy as 20 having a content of TaC/NbC this is intended to convey that the alloy contains either or both the compounds TaC and NbC, and that where a percentage figure is given against the expression TaC/NbC this refers to the content of (TaC+NbC) in the alloy.

The bonding metal usually consists substantially entirely of Co and/or Ni. I have found that with the relatively high proportion of TiC included in the alloy of the present invention it may be advantageous to use Ni 25 as a bonding metal, as Ni has a greater capacity for dissolving TiC than has Co.

In comparison with known hard metal alloys for finishing materials such as steel the alloy of this invention has an increased amount  $\beta$ -phase. This has been shown to 30 be of importance for obtaining an increase in the strength of the alloy whilst maintaining or even increasing the resistance to wear, that is to say resistance against wear as well as cratering. In previously known hard metals for the purpose specified, the amount of  $\gamma$ -phase has been less than  $100 - 2\beta$ , whilst the amount of bonding metal has been considerably below the limits specified for this invention.

For obtaining the unusual properties for the hard metal alloy according to this invention the composition of the 35 alloy is of great importance. The limits of the values of the components have been indicated above. It has usually proved to be advantageous if the hard metal contains up to 5% by weight (preferably between 1 and 3% by weight) of TaC/NbC. The amount of the bonding metal is preferably chosen within the range 8-11% by weight and often within the range 9-10.5% by weight. The content of TiC is preferably between 35 and 45% by weight and is often within the range 36-42% by weight.

55 The composition by weight of the alloys in accordance with the present invention is preferably chosen within the following limits:

|                                        |           |       |
|----------------------------------------|-----------|-------|
| TiC                                    | percent   | 36-42 |
| TaC/NbC                                | do        | 1-3   |
| Bonding metal, preferably Co and/or Ni | do        | 9-11  |
| WC                                     | remainder |       |

The invention will now be illustrated by some examples giving the approximate composition by weight for 60 certain alloys in accordance with the invention.

## Example 1

|         | Percent by weight |
|---------|-------------------|
| TiC     | 40                |
| TaC/NbC | 2                 |
| Co      | 10                |
| WC      | 48                |

## Example 2

## Percent by weight

|         |    |
|---------|----|
| TiC     | 35 |
| Co      | 9  |
| WC      | 54 |
| TaC/NbC | 2  |

The alloy consisted of about 9% by volume of  $\beta$ -phase, about 90% by volume of  $\gamma$ -phase and about 1% by volume of  $\alpha$ -phase.

The accompanying drawing shows diagrammatically the amount of wear as a function of the cutting speed for three hard metals A, B and D, the first two of which are of a known type and the last is made in accordance with the invention when turning carbon steel with a C-content of 0.84% by weight and with a hardness Nb=230. The amount of wear is defined as the maximum crater depth in microns and the cutting speed is in meters/minute. The feed was 0.51 mm./turn, the cutting depth 1.0 mm. and for all the tests which formed a basis for the curves, the cut chip length was 1000 meters.

The composition by weight of the hard metals was:

|         | A, per-<br>cent | B, per-<br>cent | D, per-<br>cent |
|---------|-----------------|-----------------|-----------------|
| TiC     | 25              | 36              | 40              |
| TaC/NbC |                 | 2               | 2               |
| Co      | 6               | 6               | 10              |
| WC      | 69              | 56              | 48              |

The alloy D consisted of about 9% by volume of  $\beta$ -phase and about 91% by volume of  $\gamma$ -phase.

The diagram shows that the alloy D made in accordance with the invention had a considerably higher wear resistance than the earlier known alloys A and B. The alloy A which showed the worst wear resistance could not resist speeds of more than 190 meters/minute. It may also be mentioned that the alloys A and D showed substantially the same toughness, while the alloy B had a considerably lower toughness.

In the manufacture of alloys in accordance with the invention it has been proved to be advantageous to add titanium carbide in the form of a so-called double carbide (Ti, W) C, consisting for example 50% by weight of titanium carbide and 50% by weight of tungsten carbide. Tantalum carbide and/or niobium carbide may either be added in the form of single carbides or in the form of a solid solution (Ta, Nb) C. Of course, it is also possible to include carbides in other solid solutions, for example in the form of (Ti, Ta, W) C. The correct

proportions of these components are ground with tungsten carbide and bonding metal to a grain size which will give the sintered hard metal alloy product a grain size of preferably 2-5  $\mu$ m. After pressing portions of the powder to a suitable size and shape they are suitably sintered in a vacuum oven at about 1600° C. for about 1 hour.

I claim:

1. A sintered hard metal alloy consisting essentially of the following components in the following percentages by weight: TiC, 30 to 45%; a carbide of the group consisting of TaC and NbC, 1 to 3%; auxiliary bonding metal of the group consisting of Ni, Co and Fe, 8-11%; the remainder being substantially all WC, said alloy being further characterized in that said alloy is composed of a  $\gamma$ -phase consisting of a solid solution, in TiC, of all of the carbide of the group consisting of TaC and NbC and substantially all of the WC and an  $\alpha$ -phase consisting of the remaining undissolved WC and a  $\beta$ -phase consisting of auxiliary bonding metal, the amount of the  $\beta$ -phase thereof and the amount of the  $\gamma$ -phase thereof being related to one another by the relationship

$$100 - \beta \geq \gamma \geq 100 - 1.5\beta$$

and the sum of the amounts of the three phases  $\alpha$ ,  $\beta$  and  $\gamma$  equals 100, where  $\alpha$ ,  $\beta$  and  $\gamma$  represent the amounts of the respective phases in volumes percent.

2. A sintered hard metal alloy according to claim 1, wherein the amount by weight of the TiC content is within the range 35-45%.

3. A sintered hard metal alloy according to claim 1, wherein the bonding metal substantially consists of nickel and the content thereof is within the range 9-10.5%.

4. A sintered hard metal alloy according to claim 1 and of the following composition by weight: 36-42% TiC, about 2% of a carbide selected from the group consisting of tantalum carbide and niobium carbide, 9-10.5% Ni; remainder substantially all WC.

5. A sintered hard metal alloy according to claim 1, wherein the bonding metal substantially consists of cobalt and the content thereof is within the range 9-10.5%.

6. A sintered hard metal alloy according to claim 1 and of the following composition by weight: 36-42% TiC, about 2% of a carbide selected from the group consisting of tantalum carbide and niobium carbide, 9-10.5% Co; remainder substantially all WC.

## References Cited in the file of this patent

Schwarzkopf: "Powder Metallurgy, Its Physics and Production," Macmillan Co., New York (1947), pp. 208-211.